

# UNITED STATES PATENT OFFICE

ROBERT A. CARTER, JR., OF NEW YORK, N. Y.

## SMOKELESS BRIQUET AND PROCESS OF MAKING SAME.

968,123.

Specification of Letters Patent. Patented Aug. 23, 1910.

No Drawing.

Application filed December 14, 1909. Serial No. 532,999.

*To all whom it may concern:*

Be it known that I, ROBERT A. CARTER, Jr., a citizen of the United States, and a resident of New York city, in the county of 5 New York and State of New York, have invented certain new and useful Improvements in Smokeless Briquets and Processes of Making the Same, of which the following is a specification.

10 This invention relates to smokeless briquets and the process of making the same out of substantially a waste product, or a by-product of comparatively little value, in the manufacture of gas for domestic and 15 manufacturing purposes.

The coke which is obtained from the destructive distillation of coal in the manufacture of gas is more or less broken and pulverized as the result of handling to get 20 the same from the retorts to the consumer. This coke is quite brittle and portions of it are pulverized or broken into fine particles by rubbing against each other and against the conveyer, or other means used to transport it to the proper bins prior to its sale. 25 This fine coke, which is formed of small particles, is screened from the other coke to make the latter merchandisable, and is a by-product of very little value as compared with 30 the coke. In some instances there is no sale for these screenings or "breeze" as known in the art, while in other localities there is a market for it at a very low figure. By my invention I take this breeze or screenings and mix with it any suitable partially 35 volatilizable binder to form a briquet and then subject the briquet to volatilization to drive out all volatile matter and gases of the binder, the resulting briquet being practically smokeless.

If the briquets are not subjected to volatilization the gases of the binder are given off quickly when the briquets are fed to a boiler or a stove, resulting in the smoke or 45 gases being under considerable pressure which, when used for instance in domestic service, will cause the smoke and volatile gases to be forced out through the crevices and cracks of the stove besides forming soot 50 within its drafts, passages and connecting pipes. This objection applies also more or less to the use of such briquets as fuel for boilers for manufacturing purposes.

By my invention I take the breeze or 55 screenings of coke which is approximately

10% to 20% or more, of the total output of coke, depending upon how it is handled, and mix with it any suitable binder to make the briquets which may be given any desired shape or contour. In practice I have 60 found that a very good binder is ordinarily coal tar pitch, very satisfactory results being obtained with pitch which is known as 170°, the same being its melting point, though of course, it is to be understood that 65 my invention is not limited to this or any other particular form of binder. I preferably mix the binder in a condition sufficiently fluid to enable it to be at least partially absorbed by the porous particles of 70 the breeze and when the briquets are subsequently coked this absorption insures a permanent adhesion between the coke particles and the binder whereby a briquet substantially uniformly coked throughout is 75 produced and crumbling and waste prevented. After the breeze or screenings are mixed with the suitable binder and given a proper shape or configuration, depending upon the use to which it is to be put, I 80 place the resulting briquets in a volatilizer and subject them to sufficient heat to drive off substantially all the volatile matter of the binder. This leaves the resulting briquets more or less porous and if the volatilization is continued, the relatively small portion of the binder, which is left in the briquet is very hard. In this second treatment of the screenings or breeze what little volatile matter remains in it from its first 85 destructive distillation is driven off with the volatile matter of the binder, the resulting briquet being comparatively firm and burning substantially without smoke.

I have described this invention in connection with one manner of practicing the same but it is to be understood that my invention is not to be limited to the details here set out for what is claimed as new and what it is desired to secure by Letters Patent is 90 set forth in the appended claims.

1. A porous smokeless briquet comprising coke screenings or breeze and a volatilized binder formed from coal tar pitch of substantially 170° melting point combined with 100 the breeze and coked.

2. The method of making smokeless briquets consisting in mixing ordinary coal tar pitch of substantially 170° melting point with the breeze or coke screenings and sub- 110

jecting the same to volatilization to drive off the volatile matter in the said coal tar pitch.

3. A substantially smokeless briquet comprising coke screenings or breeze and a volatilized binder at least partially absorbed by the breeze and having its unvolatilized portion or base forming a permanent adhesion between the coke particles, insuring the briquet being uniformly coked throughout and preventing crumbling and waste of the briquet.

4. The method of making substantially smokeless briquets consisting in mixing with breeze or coke screenings a partially volatilizable binder in a condition sufficiently

fluid to enable it to be at least partially absorbed by the porous particles of the breeze, shaping the briquets, subjecting the briquets to volatilization to drive off the volatile matter in the binder, and leaving the absorbed base or unvolatilizable portion of the binder in the briquets to form a permanent adhesion between the coke particles whereby a briquet substantially uniformly coked throughout is produced and crumbling and waste prevented.

ROBERT A. CARTER, JR.

Witnesses:

ROSE MENK,  
ALAN M. JOHNSON.